

## UNITED STATES PATENT OFFICE

2,367,511

## PHOTOGRAPHIC EMULSIONS

Wesley G. Lowe and William F. Fowler, Jr., Rochester, N. Y., assignors to Eastman Kodak Company, Rochester, N. Y., a corporation of New Jersey

No Drawing. Application April 15, 1944.  
Serial No. 531,286

5 Claims. (Cl. 95—7)

This invention relates to photographic emulsions in which a water-soluble resin made up of polyvinyl alcohol and polyvinyl acetate which has been treated with a water-soluble reaction product of formaldehyde and melamine is employed as the carrier for the light-sensitive element therein.

This application is a continuation-in-part of our application Serial No. 474,601, filed February 3, 1943.

In the manufacture of photographic emulsions in which gelatin is employed as the base, it is customary in cases where the emulsion is to be subjected to hot ferrotyping or to aqueous processing solutions under warm conditions to employ a hardener for the gelatin. By this hardening, the sticking of the emulsion to the hot ferrotyping roll is reduced or substantially eliminated and also processing of the emulsion is facilitated. In processing gelatin emulsions, it is often customary to incorporate hardening agents in the fixing solution to contribute to the hardness of the gelatin.

Recently, the use of polyvinyl alcohol or resins having a large proportion of polyvinyl alcohol has been suggested for photographic purposes, such as the carrier for a light-sensitive material. Silver halide emulsions have been referred to in which polyvinyl alcohol has been employed as the protective colloid therefor. For many purposes, however, polyvinyl alcohol or the polyvinyl acetates which are water-soluble by virtue of their polyvinyl alcohol content, have not been regarded as sufficiently resistant to the effects of water or of elevated temperatures. For instance, with photographic prints where hot ferrotyping is desirable, some hardening is necessary to prevent adhesion of the emulsion to the heated surface. It does not follow, however, that any compound that has a hardening action upon polyvinyl alcohol or water-soluble polyvinyl acetate is suitable for use in a photographic emulsion. Some compounds may be satisfactory as hardeners of polyvinyl alcohol, and yet have a desensitizing or fogging action upon the photographic emulsion. Other materials, while not causing desensitization or haziness, are not sufficiently effective as hardeners to impart the desired resistance to hot rollers.

One object of our invention is to provide a method for hardening polyvinyl acetates having a content of polyvinyl alcohol sufficient to impart water solubility when used in photographic emulsions, so as to be readily susceptible to hot ferrotyping and also to be readily susceptible to processing by means of aqueous developing and fixing solutions. Another object of our invention is to provide a method for hardening photographic emulsions in which polyvinyl alcohol or water-soluble polyvinyl acetates are employed as the carrier without causing desensitization of those

emulsions or affecting the clarity thereof. Other objects of our invention will appear herein.

Water solubility is ordinarily imparted to polyvinyl acetates by hydrolyzing those compounds to the desired degree. By hydrolyzing off some of the acetyl, polyvinyl alcohol is formed in the compound, the polyvinyl alcohol imparting water solubility. In some cases, substantially all of the acetyl is hydrolyzed off, and the resulting product is termed "polyvinyl alcohol" in commercial usage, this product ordinarily having approximately 5% polyvinyl acetate in the chemical combination. As a rule, polyvinyl acetates to a point that they contain at least 45% polyvinyl alcohol exhibit a water solubility, although obviously the viscosity of the material may alter this limit in the individual cases. Our invention applies to polyvinyl acetates which have been hydrolyzed to a sufficient extent to convert sufficient of the polyvinyl acetate to polyvinyl alcohol so that water solubility is obtained. In usual practice, the range of polyvinyl alcohol content will be from 45-100% and will include not only materials known as partially hydrolyzed polyvinyl acetates having a polyvinyl alcohol content within this range but also materials which are known as polyvinyl alcohol and are either made up wholly of polyvinyl alcohol or have but a negligible proportion of polyvinyl acetate therein.

We have found that water-soluble reaction products of formaldehyde and melamine when prepared under desirable conditions cause photographic emulsions using the above-described polyvinyl compounds as the carriers therein to harden sufficiently so that processing and ferrotyping may be carried out without detrimentally affecting either the physical or photographic properties of the product so treated. We have found that the emulsions in accordance with our invention are susceptible to the action of the hardening agents without any detrimental action either on the emulsion or any of the materials contained therein, so that a clear, transparent, photographic material results. We have found that the combining of formaldehyde and melamine to form a satisfactory hardening material should be carried out under certain prescribed conditions to obtain the most advantageous hardening of the emulsion without desensitizing it. In some cases, desensitization is not objectionable or it might even be desirable. For instance, where an emulsion is desired which is sensitive to intense light but not to ordinary light, desensitization might be desirable. As an example of photographic emulsions which may be hardened in accordance with our invention, reference may be had to U. S. Patents No. 2,276,323 and No. 2,286,215 of Wesley G. Lowe.

To obtain a hardening agent in which the desensitizing action is reduced to a minimum or



The terms "2/3 complete" and "1/3 complete" refer to judgments based on the solubility of the emulsion in hot water. The term "complete" refers to a degree of hardness such that the emulsion did not melt on commercial hot ferro-typing.

*Example 4*

Compositions were prepared of partially hydrolyzed polyvinyl acetates as follows:

|        | Percent<br>vinyl<br>acetate | Percent<br>colloid |
|--------|-----------------------------|--------------------|
| A..... | 21.4                        | 11.60              |
| B..... | 26.6                        | 12.10              |
| C..... | 33.1                        | 12.65              |
| D..... | 43.4                        | 13.70              |
| E..... | 52.8                        | 14.60              |

In each case the colloid was dissolved in a solvent mixture of 1 part ethyl alcohol and 1 part water by volume. Besides the colloid, the solvent contained acetic acid or its salt and ethyl acetate, formed by the hydrolysis of the polyvinyl acetate and also a small amount of sodium sulphate which results from the neutralization of the sulphuric acid used as the catalyst in the polyvinyl acetate hydrolysis.

The following formula was employed for the preparation of photographic emulsions from A, B and C respectively:

30 grams of the solution of colloid were diluted with a mixture of 150 cc. of ethyl alcohol and 45 cc. of water. Into this solution held at 110° F. was run simultaneously solutions 1 and 2 with rapid stirring:

*Solution 1.*—10 grams of silver nitrate dissolved in water and made up to a volume of 20 cc.

*Solution 2.*—6.4 grams of potassium bromide, .25 gram of potassium chloride, .25 gram of potassium iodide, dissolved in water and made up to a volume of 20 cc.

To the dispersion so obtained were added 150 grams of the colloid solution. One hundred cc. of a 50% aqueous alcohol solution was added and the emulsion was sensitized, with 4 mg. of 2,3'-diethyl - 4' - methyloxathiazolo-carbocyanine iodide. Also 4% (based on the weight of resin present in the emulsion) of melamine-formaldehyde hardener was added.

The emulsions were then coated on paper and dried. After 5 days the paper was processed and was subjected to hot-ferrotyping. It was found that each of these emulsions passed through the processing baths unimpaired and that they resisted the melting action of the hot-ferrotyping. The emulsions formed showed excellent photographic qualities.

The following formula was used for the preparation of photographic emulsions from colloids D and E.

Solutions 1 and 2, as referred to above, were each diluted by the addition of 20 cc. of ethyl alcohol to each. The procedure described above was otherwise followed. After the emulsion was sensitized, 8% of melamine-formaldehyde (based on the weight of resin in the emulsion) was added. The emulsions were coated out onto paper and they were found to be sufficiently hardened to process satisfactorily after 3 days and were resistant to the solvent action of hot water and to the melting action of hot-ferrotyping after 10 days.

The time of hardening of the emulsion in accordance with my invention decreases with

an increased proportion of the hardening agent. It is desirable in practical operations that at least 4% of hardener based on the resin in the emulsion be employed to assure hardening within a few days. However, my invention contemplates polyvinyl acetate emulsions broadly having the vinyl acetate proportion specified with various proportions of melamine-formaldehyde hardener, as it is optional with the operator whether to use a proportion of hardener which will give optimum properties within a few days or to use a smaller proportion of hardener and increase the time of storage before the emulsion is used. It is desirable to employ greater proportions of hardener with polyvinyl acetate emulsions having vinyl acetate contents in the higher portion of the specified range than with those emulsions in which the vinyl acetate content is in the lower part of the range. The percentage of hardener added throughout this application refers to the percentage by weight of formaldehyde used in making the hardener employed to the weight of polyvinyl acetate in the emulsion. Ordinarily, it is desirable that no more than 10% of the hardener be added to the emulsion. In cases where the amounts of formaldehyde, employed in preparing the hardener, are over 6 moles of formaldehyde to 1 mole of melamine, the ratio of formaldehyde to polyvinyl acetate in hardening the emulsion is figured on the basis of 6 moles of formaldehyde to 1 of melamine in preparing a hardener. In other words, in preparing a hardener where the mole ratio of formaldehyde to melamine is 6 or less the relation of hardener to polyvinyl acetate employed in making photographic emulsions is figured on the percentage of formaldehyde used in making the hardener to the polyvinyl acetate in the emulsion. When more than 6 moles of formaldehyde are employed to 1 of melamine in making the hardener, the percentage of hardener to polyvinyl acetate in the emulsion is figured on the basis of 6 moles of formaldehyde to 1 of melamine in the hardener preparation.

The term "water-soluble polyvinyl acetate" is employed in this application to refer to polyvinyl acetates having a polyvinyl alcohol content in sufficient amount to render the material water-soluble. This term includes materials which are referred to in commercial practice as polyvinyl alcohols.

I claim:

1. A photographic emulsion containing as the protective colloid for the photo-sensitive element therein a water-soluble hydrolyzed polyvinyl acetate and a water-soluble melamine-formaldehyde hardener resulting from reacting together one mole of melamine and 1 to 10 moles of formaldehyde.

2. A photographic emulsion containing as the protective colloid for the photo-sensitive element therein a water-soluble hydrolyzed polyvinyl acetate and a water-soluble melamine-formaldehyde hardener resulting from reacting together 1 mole of melamine and 3 moles of formaldehyde.

3. A method of hardening a photographic emulsion containing water-soluble hydrolyzed polyvinyl acetate as the carrier therein, which comprises mixing together 1 mole of melamine and 1 to 10 moles of formaldehyde in aqueous solution at a pH of 3.5-9 and a temperature of 60-85° C. and 0 to 2 hours after the melamine dissolves, cooling the mass to below 60° C. followed by adding the mass to the photographic emulsion.

4. A method of hardening a photographic emul-

sion containing water-soluble hydrolyzed polyvinyl acetate as the carrier therein, which comprises mixing together 1 mole of melamine with 3 moles of formaldehyde in aqueous solution at a temperature between 75° and 85° C. and pH between 6 and 8 until the melamine dissolves, cooling the mass to room temperature and incorporating it in the photographic emulsion in the proportion of at least 0.5% of formaldehyde employed in making the hardener, based on the water-soluble hydrolyzed polyvinyl acetate present in the emulsion.

5. A method of hardening a silver halide emulsion in which water-soluble hydrolyzed polyvinyl acetate is present as the protective colloid for the silver halide, which comprises mixing together 1 mole of melamine and 1 to 10 moles of formaldehyde in aqueous solution at a pH of 3.5 to 9 and a temperature of 60-85° C. and 0 to 2 hours after the melamine dissolves, cooling the mass to below 60° C. followed by adding the mass to the photographic emulsion.

WESLEY G. LOWE  
WILLIAM F. FOWLER, Jr.